

# UNITED STATES PATENT OFFICE.

WINFIELD SCOTT POTTER, OF PITTSBURGH, PENNSYLVANIA.

## HEAT TREATMENT OF MANGANESE STEEL.

1,123,003.

Specification of Letters Patent. Patented Dec. 29, 1914.

No Drawing.

Application filed April 17, 1914. Serial No. 832,527.

To all whom it may concern:

Be it known that I, WINFIELD SCOTT POTTER, a citizen of the United States, residing at Pittsburgh, Allegheny county, State of Pennsylvania, have invented certain new and useful Improvements in Heat Treatment of Manganese Steel; and I do hereby declare the following to be a full, clear, and exact description of the invention, such as will enable others skilled in the art to which it appertains to make and use the same.

The present invention relates to a method of heat treating rolled, forged and otherwise wrought shapes of manganese steel; that is to say, steel containing over 5% of manganese, with or without silicon or alloying metals such as chromium or nickel, and containing any suitable proportion of carbon (for instance from .25% to 2.25% of carbon).

The product obtained by the practice of the invention has not only the well-known toughness and strength of manganese steel, but, in addition thereto, is further insured against risk of breakage in service for the reason that in all cases the peculiar condition of manganese steel which may be designated the "crackled" condition is avoided.

In accordance with the improved method of heat treatment, herein described, the manganese steel product may be given the maximum attainable combination of ultimate strength and elastic limit, together with a ductility which is nearly the greatest ductility obtainable by heat treatment; or, the manganese steel product may be given the maximum attainable ductility with nearly the highest possible combination of ultimate strength and elastic limit obtainable by heat treatment alone.

I have discovered a critical range of temperatures terminating, during the heating of manganese steel of ordinary composition, at about 825° C.-850° C., and having, in heating, a low limit of about 710° C. This critical range corresponds to the absorption (that is to say, the solid re-solution by the mixed crystals of the metal) of the carbids and carbon-containing alloys which separate within the mass while the mass is cooling through and below said critical range, and, while the mass is either cooling or being heated at temperatures below said range.

I have found that when the manganese steel is heated to a temperature at, or just

above the upper limit of this critical range, the steel is given a new and very fine-grained structure, and if it is then water-quenched (in order to make permanent the condition due to heating), it does not tend to rupture between the grains, when subjected to shock or strain; on the contrary, if then broken, it presents, largely or entirely, a fracture that may be called "silky," and not a granular fracture such as occurs in the steel in which the grain adhesion is weaker than the cohesive strength of the metal in the grains. I have also found the greatest strength of the manganese steel due to heat treatment is attained by heat treatment at a temperature just above the critical range referred to, and that the greatest elongation or ductility of the steel is obtained by heating it at about 25° C.-50° C., above the upper limit of the critical range.

Furthermore, I have found that when the manganese steel is heated to any temperature from the upper end of the hereinbefore described critical range, up to a limit of about 100° C.-125° C., above the critical range, the steel still has a strong adhesion between the grains, which adhesion is about equal to the cohesive strength of the metal in the grains. I have also found that when the manganese steel is heated to a temperature higher than 125° C., above the said critical range, the grain adhesion is greatly decreased, and that the quality of ordinary manganese steel when heat treated, for instance, at temperatures of say 975° C.-1100° C. is much inferior to the qualities obtainable by heat treatment at temperatures between the upper limit of the critical range and 100° C.-125° C. above the critical range. For instance, wrought manganese steel, in which the critical range is passed at a temperature of 850° C., and which is water-quenched before the heat treatment has carried it above 875° C., has an ultimate strength of say 160,000 pounds per square inch, and an elongation of about 55%.

If heat treated at about 900° C., the steel has an ultimate strength of about 150,000 pounds per square inch and an elongation of about 60%. If heat treated at about 975° C., the steel has an ultimate strength of about 130,000 pounds per square inch and an elongation of about 55%. When heat treated at about 1025° C., the steel has an ultimate strength of about 120,000 pounds

per square inch, and an elongation of about 40%. When heat treated at temperatures above 975° C., the stretched manganese steel bar usually cracks between the grains, more or less, exhibiting the state of the steel which I call the "crackled" condition,—a condition undesirable for the resistance of frequently applied strains such as those which it is necessary for steel to resist in engineering service.

In the practice of my improved method of heat treating wrought manganese steel, the wrought product, finished as to form, is placed in a furnace which is supplied, as nearly as practicable, with a neutral or non-oxidizing atmosphere or medium, and is therein heated either rapidly or slowly to a predetermined maximum temperature, dependent upon the analysis of the metal, (that is, at a higher or lower temperature in proportion to the percentage of manganese) which determines the location of the critical point, (at the upper limit of the hereinbefore mentioned critical range) at which critical point the metal is completely transformed into the uniform austenitic state. The maximum temperature to be selected for the heat treatment will also depend upon the stiffness or ductility desired in the product. For example, if a product is being heat treated in order to impart to it the ductility suitable for cold drawing, cold stamping, cold pressing, or otherwise cold forming, where a maximum of ductility is desirable, the maximum temperature of the heat treatment will be located at about 25° C.—100° C., above the austenite-forming critical range. If, however, the maximum of strength and stiffness combined with a moderately high ductility is desired, the manganese steel product is heated to, or slightly above the upper limit of the critical range. When the greatest stiffness with less than the greatest obtainable ultimate strength and ductility is preferred, the product is heated to a temperature at, or slightly below, the upper limit of the critical range.

In contrast to previously proposed methods of heat treating manganese steel, the steel is preferably held for some time in the furnace, at or about the maximum temperature employed in the heat treatment. In fact, it is only by permitting the steel to come to a state of equilibrium at the maximum temperature of the heat treatment, that the fine-grained uniform austenite state of the metal, which is both strong and tough, can be produced at, or slightly above, the upper limit of the critical range. By using suitable means of avoiding surface oxidation of the manganese steel product, I have found it possible to hold the steel in the furnace, at the maximum temperature employed, for a period of one hour or more, without loss of grain adhesion at tempera-

tures just below, at, or even 125° C. above the upper limit of the critical range; whereas, when the temperature is, for example, 150° C. or more above the upper limit of the critical range, the product can only be held in the furnace at the maximum temperature employed for such time as is necessary to impart to the metal body a uniform temperature, for the reason that, if held longer in the furnace, the grain adhesion is found to be objectionably low, beginning at the surface of the metal body and extending inward to a depth dependent upon the time during which it was held in the furnace after the uniform maximum temperature had been obtained.

It will, of course, be understood, that when the manganese steel product, in the practice of my invention, has been brought, by the heat treatment described, to the desired condition of re-solution of the separable constituents referred to, and has attained the desired condition of equilibrium, such condition is made permanent by rapidly cooling the product to ordinary temperatures,—as, for instance, by quenching the product in water.

Having thus described my invention, what I claim is:

1. The method of heat treating a wrought manganese steel product, comprising heating the said product to a temperature substantially as high as that of the upper limit of the critical range for the re-solution of the constituents which have separated out from the mixed crystals of the manganese steel product, retaining the product at substantially the maximum temperature of the heat treatment until the metal of the product is brought to a state of equilibrium, and, finally, rapidly cooling the product to ordinary temperature.

2. The method of heat treating a wrought manganese steel product, comprising heating the said product to a temperature slightly above that of the upper limit of the critical range for the re-solution of the constituents which have separated out from the mixed crystals of the manganese steel product, retaining the product at substantially the maximum temperature of the heat treatment until the metal of the product is brought to a state of equilibrium, and, finally, rapidly cooling the product to ordinary temperature.

3. The method of heat treating a wrought manganese steel product, comprising heating the said product to a maximum temperature within a range of 125° C. above the upper limit of the critical range for the re-solution of the constituents which have separated out from the mixed crystals of the manganese steel product, retaining the product at substantially the maximum temperature of the heat treatment until the metal

of the product is brought to a state of equilibrium, and, finally, rapidly cooling the product to ordinary temperature.

4. The method of heat treating a wrought manganese steel product, comprising heating the said product to a temperature substantially as high as 825° C.-850° C., retaining the product at substantially the maximum temperature of the heat treatment until the metal of the product is brought to a state of equilibrium, and, finally, rapidly cooling the product to ordinary temperature.

5. The method of heat treating a wrought manganese steel product, comprising heating the said product to a temperature slightly above 825° C.-850° C., retaining the product at substantially the maximum temperature of the heat treatment until the metal of the product is brought to a state of

equilibrium; and, finally, rapidly cooling the product to ordinary temperature.

6. The method of heat treating a wrought manganese steel product, comprising heating the said product to a temperature within a range of 125° C. above 825° C.-850° C., retaining the product at substantially the maximum temperature of the heat treatment until the metal of the product is brought to a state of equilibrium, and, finally, rapidly cooling the product to ordinary temperature.

In testimony whereof I affix my signature, in presence of two witnesses.

WINFIELD SCOTT POTTER.

Witnesses:

M. A. BILL,  
R. MONTGOMERY.